

July 28, 1964

E. H. LAND

3,142,566

PHOTOGRAPHIC PROCESS

Original Filed May 7, 1958

FIG. 1



FIG. 2



INVENTOR.  
*Edwin H. Land*  
BY  
*Brown and Melville*  
*and*  
*Gerald Altman*  
ATTORNEYS

## 1

3,142,566

## PHOTOGRAPHIC PROCESS

Edwin H. Land, Cambridge, Mass., assignor to Polaroid Corporation, Cambridge, Mass., a corporation of Delaware  
Continuation of application Ser. No. 733,754, May 7, 1958. This application Feb. 14, 1962, Ser. No. 176,844  
7 Claims. (Cl. 96—61)

The present invention relates to novel photographic processes, and more particularly to novel processes for developing latent images formed in photoexposed photosensitive elements.

The primary object of the present invention is the novel use of photographic elements comprising photosensitive materials formed, at least in part, by the vacuum deposition of their components upon their support. It has been found that such extremely thin and protective-colloid-free photosensitive materials possess peculiar characteristics that unexpectedly make feasible the development of latent images by the application of heat.

Other objects of the invention will in part be obvious and will in part appear hereinafter.

The invention accordingly comprises the process possessing the several steps and the relation and order of one or more of such steps with respect to each of the others, which are exemplified in the following detailed disclosure, and the scope of the application of which will be indicated in the claims.

For a fuller understanding of the nature and objects of the present invention, reference should be had to the following detailed description taken in connection with the accompanying drawing wherein:

FIGURE 1 shows successive, exaggerated diagrammatic cross-sectional views of materials being treated in accordance with the present invention; and

FIGURE 2 shows successive, exaggerated cross-sectional views of the product of the process of FIGURE 1 being used in accordance with the present invention.

Generally, the process of the present invention herein disclosed is based upon the production of a photosensitive stratum by vacuum depositing at least a metal of a photosensitive salt on a support and then subjecting the metal on the support to halogen vapor. The support, for example, is composed of a suitable plastic such as hydrolyzed cellulose acetate or a suitable paper such as baryta paper.

The step of vacuum depositing involves either evaporating or sputtering at pressures below one hundred microns of mercury, and usually within the range of from 0.1 to 100 microns of mercury, these pressures being produced by continuous evacuation to ensure the rapid removal of any gases produced during the vacuum deposition process. The metallic distribution of the stratum initially formed preferably is in sufficient concentration per unit area to give rise to an optical transmission of at most 40%. Unusually satisfactory results are achieved when the metal distribution includes both gold and silver deposited in either sequence or together. Best results are achieved when the silver is vacuum deposited in a concentration that by itself would give rise to an optical transmission of from 10% to 30%, the gold is deposited in a concentration that by itself would give rise to an optical transmission of from 10% to 30% and the gold and silver are deposited in concentrations which together give rise to an optical transmission of from 0.01% to 1.0%.

Halogenation is effected by subjecting the metallic stratum produced in the foregoing way to the vapor of elemental halogen, e.g. chlorine, bromine, iodine or combinations thereof or to volatile halogen salts, e.g. hydrogen bromide, hydrogen iodide or combinations thereof at a suitable temperature, for example, room temperature.

## 2

The metallic stratum, preferably, is subjected to the halogen vapor for a period sufficient to effect substantially complete halogenation, a condition that is indicated when the optical transmission of the stratum has increased substantially to between 85% and 100%.

In accordance with the present invention, development of a latent image in a photosensitive stratum produced in the foregoing way, by virtue of its peculiar structure, is effected by the application of heat, for example, the generation, by infrared or ultra high frequency radiation, of temperatures elevated above room temperature for periods necessary to effect development.

## Example

FIGURE 1 illustrates the production of a photosensitive element in accordance with the present invention. As shown, the support is a hydrolyzed cellulose acetate sheet 20, approximately 1 millimeter thick, 3 inches wide and 6½ inches long. First, 5 milligrams of gold is evaporated uniformly onto the support to form a gold stratum 22. The resulting optical transmission of the strip is 20%. Then 5 milligrams of silver is evaporated onto the support to form a gold-and-silver stratum 24. The resulting optical transmission is 0.06%. Finally, gold-and-silver stratum 24 is subjected in a closed jar to the vapor of a quantity of hydrogen bromide until an optically clear photosensitive stratum 26 is formed. Photosensitive stratum 26 is characterized by low photographic speed, negligible graininess and a long soft curve. The photosensitive element of FIGURE 1, after being photoexposed, is subjected to a temperature of approximately 100° F. A negative print of delicate gradation is produced in approximately fifteen minutes. The print of the above example may be fixed by reacting its unreduced silver with a fixing vapor, e.g. hydrogen sulfide, to form a stable silver salt.

This application is a continuation of my application Serial No. 733,754, filed May 7, 1958.

Since certain changes may be made in the above process without departing from the scope of the invention herein involved, it is intended that all matter contained in the above description and shown in the accompanying drawing shall be interpreted as illustrative and not in a limiting sense.

## What is claimed is:

1. A process of forming photographic negative images comprising the steps of (a) forming a photosensitive, vacuum deposited metallic halide stratum including at least silver halide, by vacuum depositing said metals, including silver, upon a support in a concentration providing a metallic stratum having an optical transmission of from about 0.01% to about 1.0%, halogenating said vacuum deposited metallic stratum by contacting said metallic stratum with halogen vapors provided with a member of the group consisting of elemental chlorine, elemental bromine, elemental iodine, and volatile salts of said elemental halogens for a time sufficient to provide a halogenated metallic coating having an optical transmission of from about 85% to about 100%, (b) photoexposing the thus-prepared photosensitive vacuum deposited metallic halide stratum, and (c) developing said exposed photosensitive vacuum deposited metallic halide stratum to a visible negative image by subjecting said stratum to heat above room temperature, said application of heat being the sole means of effecting said development.

2. The process of claim 1, wherein said metallic stratum includes gold and silver, each of said gold and silver being deposited in a concentration which by itself would provide an optical transmission of from about 10% to about 30%, said coating of gold and silver together having a total optical transmission of from about 0.01% to about 1.0%.

3. The process of claim 1, wherein said exposed photosensitive vacuum deposited metallic halide stratum is subjected to a temperature of approximately 100° F. for a time sufficient to develop said negative image.

4. The process of claim 2, wherein said photosensitive metallic halide stratum consists of vacuum deposited silver and gold halogenated by the application of iodine vapors.

5. The process of claim 2, wherein said photosensitive metallic halide stratum consists of vacuum deposited silver and gold halogenated by the application of hydrogen bromide vapors.

6. The process of claim 1, including the step, after said heat development, of converting unexposed and undeveloped silver halide to a light stable silver salt.

7. The process of claim 1, including the step, after

4  
said heat development, of reacting unexposed and undeveloped silver halide with hydrogen sulfide vapors.

References Cited in the file of this patent

UNITED STATES PATENTS

|           |               |                |
|-----------|---------------|----------------|
| 2,153,628 | Knoll         | April 11, 1939 |
| 2,239,452 | Williams      | Apr. 22, 1941  |
| 2,439,983 | Morgan et al. | Apr. 20, 1948  |

OTHER REFERENCES

10 Yamada et al.: Chem. Abstracts, vol. 50, pp. 11147-8.  
(Copy in Sci. Lib.)

Glafkides: Photographic Chemistry, I, Fountain Press, London 1958, p. 319.

15 Humphrey: American Handbook of the Daguerreotype, 5th ed., pub. by S. D. Humphrey, N.Y., 1958, pp. 35-37, 158 and 159. (Copy in Sci. Lib.)

UNITED STATES PATENT OFFICE  
CERTIFICATE OF CORRECTION

Patent No. 3,142,566

July 28, 1964

Edwin H. Land

It is hereby certified that error appears in the above numbered patent requiring correction and that the said Letters Patent should read as corrected below.

Column 2, line 54, for "with", second occurrence, read  
-- by --; lines 69 and 71, for "transmision", each occurrence,  
read -- transmission --.

Signed and sealed this 12th day of January 1965.

(SEAL)

Attest:

ERNEST W. SWIDER  
Attesting Officer

EDWARD J. BRENNER  
Commissioner of Patents